

L. W. CHUBB.  
SERIES TRANSFORMER.  
APPLICATION FILED APR. 12, 1915.

1,277,384.

Patented Sept. 3, 1918.



Fig. 3.

6% Nickel 18  
Iron 17  
19



Fig. 2.

WITNESSES:

Fred A. Lind  
Geo. W. Hansen.

INVENTOR

Lewis W. Chubb  
BY  
Chesty G. Carr  
ATTORNEY

# UNITED STATES PATENT OFFICE.

LEWIS W. CHUBB, OF EDGEWOOD PARK, PENNSYLVANIA, ASSIGNOR TO WESTINGHOUSE ELECTRIC AND MANUFACTURING COMPANY, A CORPORATION OF PENNSYLVANIA.

## SERIES TRANSFORMER.

1,277,384.

Specification of Letters Patent. Patented Sept. 3, 1918.

Application filed April 12, 1915. Serial No. 20,686.

To all whom it may concern:

Be it known that I, LEWIS W. CHUBB, a citizen of the United States, and a resident of Edgewood Park, in the county of 5 Allegheny and State of Pennsylvania, have invented a new and useful Improvement in Series Transformers, of which the following is a specification.

My invention relates to electrical apparatus and it has special reference to series or current-type transformers which supply energy at low voltages to trip coils of circuit breakers or other devices and to electrical measuring instruments. 10 15 More particularly, my invention relates to current or series transformers which are adapted to be inserted in power circuits for supplying energy to ammeters, current coils of wattmeters or other devices, etc. 20 Power circuits that supply energy to electrical apparatus are subject to short circuits which cause abnormal electrical currents to flow over the power mains. Series or current transformers of the usual type, that are 25 inserted in such mains, are liable to injury because of the high mechanical stresses developed, in addition to, the dangerous effects arising from the abnormally high currents thus induced in the secondary windings. 30 The coils of ammeters, wattmeters, etc., connected in circuit with the secondary windings of these transformers are frequently burned out because of these high secondary currents, and the needles of such instruments are frequently damaged as a result of 35 abnormal deflections.

By means of my invention, I provide a series transformer with a core made of a magnetizable alloy which becomes substantially saturated when subjected to low magnetizing forces or magneto-motive forces of low values. It is well known that, in series 40 45 transformers, the magnetic cores are normally operated at relatively low inductions. However, when abnormally high currents, such as short circuit currents, flow through the primary windings, the magnetic cores of the usual series transformers become saturated at high magnetic inductions, there- 50 55 by inducing abnormally high currents in the secondary windings. If these usual iron magnetic cores are replaced by cores made of a material which becomes fully saturated by low magnetizing forces, the currents induced in the secondary windings un-

der abnormal conditions may be limited to safe values. For example, in transformers in which the magnetizable cores become substantially fully saturated at low magnetic inductions, currents induced in the secondary windings are limited to safe values irrespective of the value of the short-circuit currents flowing in the primary windings, the cores, in this instance, acting in a manner similar to air cores. 60 65

In the operation of a current transformer, it is desirable that, within the working range, the magnetizing current be maintained at a minimum value in order to obtain an accurate ratio of transformation, this result being attained by the use of a core member of high permeability. Furthermore, it is desirable that, under overload conditions, the secondary current be prevented from attaining excessive values, demanding a core 70 75 member of low permeability. These two apparently conflicting actions are obtainable by the use of nickel-iron alloys of such a per-cent. composition as to have a magnetizing curve rising steeply from the origin 80 and suddenly turning to a direction parallel to the axis of abscissae. By so designing the core member that, within the working range, the magnetization is not carried beyond the knee, the desired accuracy in the 85 transformation ratio is secured and, under overload, the secondary voltage does not rise to a harmful degree.

One object of my invention is to provide a series transformer of the above-mentioned 90 character which may be used in conjunction with electrical measuring instruments and the like to protect them against the harmful effects of abnormally high currents or short-circuit currents that may flow in the 95 circuits in which the primaries of such transformers may be connected.

For a better understanding of the nature and scope of my invention, reference may be had to the following description and the 100 accompanying drawings in which Figure 1 is a view, partially in elevation, and partially in section, of a transformer embodying a form of my invention; Fig. 2 is a dia- 105 grammatic view showing the method of connecting series transformers in power circuits, and Fig. 3 is a graph showing several magnetization curves of the material from which the magnetizable cores of my trans- 110 formers are made.

In Fig. 1, the transformer shown comprises an insulating sleeve or bushing 1 which may be of any suitable structure capable of sustaining very high voltage, annular core members 2 and 3 which surround the bushing 1 and are concentrically located thereon, low-voltage coils 4 and 5 which are wound upon the core members 2 and 3, respectively, a supporting frame 6, and a spacing insulator 7. The supporting frame 6 consists of a metal box or casing which is disposed upon a pedestal 8. The insulating spacing structure 7 is mounted on the upper portion of the casing 6 and comprises a series of superposed insulating bells or caps 9 which are firmly secured together by cement. A winding 10 which constitutes the primary winding of the series transformer, consists of several turns of insulated conductor and is formed by threading the conductor back and forth through the sleeve or bushing 1 and allowing a sufficient external loop to pass over the insulating support 7. After the primary or high-tension winding 10 is threaded into place, the several turns of which it is composed are taped together and clamped to a metal cap 11 with which the insulator 7 is provided, as shown in Fig. 1. The primary winding 10 is supplied with terminals 12 and the secondary coils 4 and 5 are supplied with terminals 13.

By referring to Fig. 2, it will be seen that the secondary winding of the series transformer is inductively interlinked with the primary winding 10, the current flowing in the secondary winding normally being proportional to the current flowing in a power main 14. Under ordinary circumstances, the magnetic induction of a common core 15 is substantially low because of the equality of the opposing primary ampere-turns and the secondary ampere-turns of the coils constituting the series transformer. Inasmuch as the core 15 of my transformer which corresponds to the core members 2 and 3 of Fig. 1, is made of a special material that becomes substantially fully saturated at a relatively low magnetic induction, as will be herein-after explained, the currents induced in a secondary winding 16 are limited to safe values, irrespective of the value of the currents flowing in the primary winding 10.

I propose to make the core members 2 and 3 of nickel-iron alloys which contain sufficient nickel to give to the alloys the magnetic properties desired. By referring to the magnetization curves of Fig. 3, it will be apparent what nickel iron alloys are suitable for use in my transformer. A magnetization curve 17 represents the relation between magnetic inductions and magnetizing forces of a sample of iron. As explained in my co-pending patent application, Serial No. 172, filed January 2, 1915, and assigned to the Westinghouse Electric and Manufac-

turing Company, the maximum degree of magnetic permeability, at high induction, may be imparted to iron and steel by the addition of amounts of nickel ranging from 1% to 7% of the alloy. Curve 18 is a representation of the magnetization curve of a nickel-iron alloy containing substantially 6% of nickel. Further increases of the percentages of the nickel content in nickel-iron alloys, up to certain percentages of nickel, 75 gives magnetization curves represented by curves 19, 20, 21 and 22. It will be noted that the curves 18, 19, 20, 21 and 22, which, of course, are only approximately plotted, have pronounced inflections at the origin, 80 or, in other words, the magnetic inductions of these samples of nickel-iron alloys are indicated as being relatively low at low magnetizing forces. Consequently, the permeability of the samples of alloys, represented by these curves, is low at low mag- 85 neto-motive forces.

As is well known in the art, nickel-iron alloys containing from substantially 23% to substantially 28% of nickel are non-magnetic, or nearly non-magnetic, and, consequently, their magnetization curves may be represented, for purposes of illustration, as corresponding, in some degree, to the base line of the X-axis of the graph in Fig. 3. 90 Moreover, the curves 19, 20, 21 and 22 conform, in some degree, to the shape of the curve 18, the samples of these alloys becoming substantially fully saturated at high magnetizing forces only. By further increasing the percentages of the nickel content in the nickel-iron alloys, the magnetization curves rise rapidly at the origin without any inflections, as indicated by curves 23, 24 and 25. In these curves, it will be 100 noted that the samples of nickel-iron alloys become substantially fully saturated at low magnetic inductions when subjected to relatively low magnetizing forces. Alloys having characteristic curves similar to the mag- 110 netization curves 23, 24 and 25 are suitable for cores in my transformers because these curves lack the inflections at the origin that are indicated by the curves 18, 19, 20, 21 and 22, and indicate that the maximum permeability of the alloys containing nickel contents above 29% occurs at low magnetizing forces. Moreover, the shape of these curves conforms, in some degree and in the regions of relatively high magnetizing forces, to 120 curve 26 which represents the magnetization curve of nickel. Curve 25 represents the magnetization curve of an iron-nickel alloy containing about 35% nickel. This curve represents sufficiently well for the 125 purpose of illustration, the magnetization curve of those nickel-iron alloys in which the nickel content exceeds substantially 29% nickel, and which are desirable for use in cores of my transformers. It is well known 130

that a complete series of these magnetization curves indicates that the magnetic induction of those alloys containing above 29% nickel reaches a maximum value when 5 the nickel content is substantially 46%–47%. Further increases in the nickel content above 46% or 47% cause the magnetization curves of the nickel-iron samples to approach that of curve 26 which, as above 10 mentioned, is a magnetization curve of nickel.

It will be apparent from the foregoing that those nickel-iron alloys containing at least 29% nickel and, preferably, about 33% 15 to 35% nickel, are highly desirable for use as magnetizable cores of series transformers. The permeability of these nickel-iron alloys, at low magnetizing forces, is substantially constant and reaches a maximum value at 20 very low magnetizing forces. Therefore, such nickel-iron alloys are desirable for use in series transformers. Moreover, these alloys become substantially fully saturated at relatively low magnetic induction when subjected to low magnetizing forces, as is indicated by the magnetization curves 23, 24 25 and 25. Since cores, constructed of nickel-iron alloys containing over 29% nickel and less than 50% nickel, become fully saturated 30 at low magnetic inductions and when subjected to low magneto-motive forces, it will be seen that the currents induced in the secondary winding 16 will be limited to safe values, irrespective of the values of the currents flowing in the primary windings 10 of 35 the series transformer.

Of course, it will be understood that the nickel-iron alloys employed in my series transformer must be heat-treated or annealed in a proper manner. The heat treatments which produce alloys that give magnetization curves similar to curves 22, 23, 24 and 25 of Fig. 3, are those between 600° to 1000° centigrade. The claims appended 40 herewith are to be interpreted in accordance with the proper heat treatments being imparted to the alloys. Again, impurities in the alloys may cause a variation of a few per cent. of the nickel content contained in the 45 alloys, but I desire to claim those nickel-iron alloys which have magnetization curves such as are represented by curves 22, 23, 24 and 25 of Fig. 3.

While I have shown and described a particular type of transformer, it will be apparent to those skilled in the art that any

type of transformer may be used in which the core members comprise nickel-iron alloys that contain over 29% nickel. The nickel content may be varied according to the particular uses to which the transformers are to be employed, but I desire to claim, for use in transformers, all those nickel-iron alloys which contain nickel contents above those contained in the non-magnetic nickel-iron 60 alloys. 65

I claim as my invention:

1. A series transformer having a primary coil, a secondary coil, and a magnetizable core interlinking both of said coils which 70 comprises a nickel-iron alloy containing over 29% nickel.

2. A series transformer having a primary winding, a secondary winding, and a common magnetizable core therefor, said 75 core comprising a nickel-iron alloy containing over 29% nickel.

3. A series transformer having a primary winding, a secondary winding, and a common core therefor, said core comprising 80 a nickel-iron alloy containing nickel in excess of that contained in the non-magnetic nickel-iron alloys.

4. A series transformer having a primary winding, a secondary winding, and a common core therefor, said core comprising 85 nickel substantially in excess of that contained in the nickel-iron alloys of low permeability.

5. A series transformer having a primary winding, a secondary winding, and a common core therefor, said core comprising 90 a nickel-iron alloy containing at least 29% nickel.

6. A series transformer having a primary winding, a secondary winding, and a common core therefor, said core comprising 95 a nickel-iron alloy containing substantially 33% to 35% nickel.

7. A series transformer having a primary winding, a secondary winding, and a common core therefor, said core comprising 100 a nickel-iron alloy which contains a sufficiently high nickel content to become substantially fully saturated at low magnetic induction when subjected to low magnetizing 105 forces.

In testimony whereof, I have hereunto subscribed my name this 31st day of March, 1915.

LEWIS W. CHUBB.